

## UNITED STATES PATENT OFFICE.

ARMAND DE WAELE, OF LONDON, ENGLAND, ASSIGNOR TO D. GESTETNER, LIMITED, OF LONDON, ENGLAND.

PRODUCTION OF STENCILS FOR USE IN DUPLICATING MANUSCRIPT AND TYPE-WRITTEN DOCUMENTS, DRAWINGS, AND THE LIKE.

No Drawing. Application filed November 21, 1923. Serial No. 676,178.

To all whom it may concern:

Be it known that I, ARMAND DE WAELE, a subject of the King of Great Britain and Ireland, and residing at 29 Belmont Avenue, Palmers Green, London, N. 13, England, have invented certain new and useful improvements in and relating to the production of stencils for use in duplicating manuscript and typewritten documents, drawings, and the like, of which the following is a specification.

This invention relates to the production of stencils for use in duplicating manuscript and typewritten documents, drawings and the like, and particularly to the type of stencil in which a porous support, such as yoshino paper, is provided with a stencil layer including an organic colloid, for instance a coagulated protein, which does not need moistening in order to soften the coating composition prior to cutting the stencil.

Certain difficulties arise in the production of stencils of this kind, the main difficulty being due to the fact that comparatively few tempering agents, the presence of which in the stencil layer is, generally speaking, (if not invariably) necessary, have hitherto been able to be brought into sufficiently intimate association with the colloid.

The choice of the tempering agents has therefore been limited to such as when dissolved in suitable organic solvents can be incorporated in the composition used for coating or can be emulsified and in the form of emulsions mixed with the "solution" of the main colloid constituent of the coating composition.

In some cases, however, it has been proposed to convert the tempering agent into a water-soluble or water-emulsifiable derivative which can be mixed with the solution of the colloid and optionally be subsequently decomposed as, for instance, in the operation of coagulating the protein.

The present invention is based upon the observation that tempering agents which are not soluble in or emulsifiable with a "solution" of the colloid or in the medium in which the colloid is dispersed can by mechanical means be brought to the desired degree of dispersion through the coating composition.

In other words, the invention is based upon the observation that by subjecting a disperse system comprising an organic colloid capable of forming a coherent gel together with a tempering agent insoluble in the medium in which the organic colloid is dispersed to purely mechanical treatment, the tempering agent may be brought to the desired degree of dispersion through the organic colloid disperse.

The degree of dispersion of the tempering agent in the composition used in forming the stencil layer should be preferably that which is regarded as characteristic of the division of the disperse phase in colloidal solutions.

As indicative of the treatment necessary, it may be remarked that the organic colloid disperse and the tempering agent may be passed together between surfaces spaced apart about 0.007 of an inch and moving relatively to one another at the rate of 17,000 to 18,000 feet per minute.

Thus, in order to secure the desired degree of dispersion a device comprising discs, the faces of which are spaced 0.007 inches apart, fourteen inches in diameter and rotated relatively to one another at a speed of 5,000 revolutions per minute, may be employed.

The immediate effect to be secured is similar to that secured in homogenizing milk, the ultimate result being similar also.

While in accordance with the present invention the desired degree of dispersion of the tempering agent may be secured purely by mechanical means or mechanical treatment and the employment of stabilizing agents, dispersants and emulsifying agents entirely dispensed with, such aids to securing the desired degree of dispersion of the tempering agents may be made use of.

Thus, for instance, pigments or other solids may be employed as ancillary dispersion means or stabilizers.

Inorganic materials capable of forming with the dispersion medium for the colloid, colloid sols or colloidal "solutions" or absorbing many times their weight of the disperse medium forming gels, may conveniently be employed and as examples of such materials highly colloidal clays may be specified. Such materials of the char-

acter indicated as are negatively charged, appear to be most suitable when, for instance, the disperse medium is water.

The material known as "bentonite," deposits of which occur in the State of Wyoming, United States of America, and in Alberta, Canada, is an example.

This material, dried at 110° C., has the following chemical composition:—

|    |                                                             |        |
|----|-------------------------------------------------------------|--------|
| 10 | Silica (SiO <sub>2</sub> )                                  | 57.98% |
|    | Ferrous oxide (FeO)                                         | 0.12%  |
|    | Ferric oxide (Fe <sub>2</sub> O <sub>3</sub> )              | 3.80%  |
|    | Alumina (Al <sub>2</sub> O <sub>3</sub> )                   | 22.46% |
| 15 | Lime (CaO)                                                  | 1.92%  |
|    | Magnesia (MgO)                                              | 3.24%  |
|    | Soda and potash (Na <sub>2</sub> O and K <sub>2</sub> O)    | 1.35%  |
|    | Sulphur trioxide (SO <sub>3</sub> )                         | 0.75%  |
|    | Loss on ignition (H <sub>2</sub> O, CO <sub>2</sub> , Org.) | 7.93%  |

20 The state of division of the material is indicated by the fact that 73.82% of the product as marketed is represented by particles less than 0.0015 mm. in diameter.

25 The addition of such materials may assist in securing or maintaining the tempering agent in the desired degree of dispersion, but it would appear that their main function is to prevent the tempering agent sweating out of the coating composition.

30 As an example of a suitable composition, the following may be given:—

150 parts by weight of a 10% solution of gelatine;

35 100 parts by weight of mineral oil of s. g. 0.85-0.90.

40 To the mixture 5 parts of bentonite previously allowed to swell or gelatinize in at least 50 parts by weight of water may be added.

45 Yoshino paper is coated with the composition in the usual manner and, after drying, the coated sheet may be treated with formaldehyde vapour if a coagulable protein constitutes the gelatinizing organic colloid in the composition.

50 When, however, seaweed jellies, such as agar-agar, carragheen moss, Irish moss, Iceland moss, Japanese isinglass or the like colloidal materials are employed, treatment with formaldehyde vapour may be omitted.

#### Claims:

55 1. The process of producing stencils for use in duplicating manuscript and typewritten documents, drawings and the like, and particularly stencils of the kind in which a porous support, such as yoshino paper, is provided with a stencil layer including a gelatinized organic colloid, for instance a coagulated protein, which does not need moistening in order to soften the coating composition prior to cutting the stencil, which comprises effecting by mechanical means the dispersion in the coating composition to the desired degree of tempering

agents which are not soluble in the medium in which the colloid is dispersed and applying said composition to a porous support.

2. The process of producing stencils for use in duplicating manuscript and typewritten documents, drawings and the like, and particularly stencils of the kind in which a porous support, such as yoshino paper, is provided with a stencil layer including a gelatinized organic colloid, for instance a coagulated protein, which does not need moistening in order to soften the coating composition prior to cutting the stencil, which comprises bringing a disperse system including an organic colloid capable of forming a coherent gel together with a tempering agent insoluble in the medium in which the organic colloid is dispersed, subjecting the mixture to purely mechanical treatment to bring the tempering agent to the desired degree of dispersion through the organic colloid disperse, and applying said composition to a porous support.

3. The process of producing stencils for use in duplicating manuscript and typewritten documents, drawings and the like, and particularly stencils of the kind in which a porous support, such as yoshino paper, is provided with a stencil layer including a gelatinized organic colloid, for instance a coagulated protein, which does not need moistening in order to soften the coating composition prior to cutting the stencil, which comprises bringing a disperse system including an organic colloid capable of forming a coherent gel together with a tempering agent insoluble in the medium in which the organic colloid is dispersed, subjecting the mixture to purely mechanical treatment to bring the tempering agent to the desired degree of dispersion through the organic colloid disperse, and applying said composition to a porous support.

40 4. The process of producing stencils for use in duplicating manuscript and typewritten documents, drawings and the like, and particularly stencils of the kind in which a porous support, such as yoshino paper, is provided with a stencil layer including a gelatinized organic colloid, for instance a coagulated protein, which does not need moistening in order to soften the coating composition prior to cutting the stencil, which comprises bringing a disperse system including an organic colloid capable of forming a coherent gel together with a tempering agent insoluble in the medium in which the organic colloid is dispersed, subjecting the mixture to purely mechanical treatment to bring the tempering agent to the desired degree of dispersion of the tempering agent in the composition used in forming the stencil layer is substantially that which is regarded as characteristic of the division of the disperse phase in colloidal solutions, and applying said composition to a porous support.

45 5. The process of producing stencils for use in duplicating manuscript and typewritten documents, drawings and the like, and particularly stencils of the kind in which a porous support, such as yoshino paper, is provided with a stencil layer including a gelatinized organic colloid, for instance a coagulated protein, which does not need moistening in order to soften the coating composition prior to cutting the stencil, which comprises bringing a disperse system including an organic colloid capable of forming a coherent gel together with a tempering agent insoluble in the medium in which the organic colloid is dispersed and an inorganic material capable of forming with the dispersion medium for the colloid colloid sols, subjecting the mix-

ture to purely mechanical treatment to bring the tempering agent to the desired degree of dispersion through the organic colloid disperse, and applying said composition to a porous support.

5. The process of producing stencils for use in duplicating manuscript and type-written documents, drawings and the like, and particularly stencils of the kind in which a porous support, such as yoshino paper, is provided with a stencil layer including a gelatinized organic colloid, for instance a coagulated protein, which does not need moistening in order to soften the 15 coating composition prior to cutting the stencil, which comprises bringing a disperse system including an organic colloid capable of forming a coherent gel together with a tempering agent insoluble in the 20 medium in which the organic colloid is dispersed and an inorganic material capable of absorbing many times its weight of the disperse medium forming gels, subjecting the mixture to purely mechanical treatment 25 to bring the tempering agent to the desired degree of dispersion through the organic colloid disperse, and applying said composition to a porous support.
6. The process of producing stencils for 30 use in duplicating manuscript and type-written documents, drawings and the like, and particularly stencils of the kind in which a porous support, such as yoshino

paper, is provided with a stencil layer including a gelatinized organic colloid, for 35 instance a coagulated protein, which does not need moistening in order to soften the coating composition prior to cutting the stencil, which comprises bringing a disperse system including an organic 40 colloid capable of forming a coherent gel together with a tempering agent insoluble in the medium in which the organic colloid is dispersed and highly colloidal clays, and applying said composition to a porous support. 45

7. The process of producing stencils for use in duplicating manuscript and type-written documents, drawings and the like, and particularly stencils of the kind in which a porous support, such as yoshino paper, is provided with stencil layer including a gelatinized organic colloid, for instance a coagulated protein, which does not need moistening in order to soften the coating composition prior to cutting the stencil, which comprises bringing a disperse system including an organic colloid capable of forming a coherent gel together with a tempering 50 agent insoluble in the medium in which the organic colloid is dispersed and bentonite, and applying said composition to a porous support. 55

In testimony whereof I have signed my name to this specification.

ARMAND DE WAELE.